

Oct. 29, 1940.

P. M. MUELLER

2,220,048

APPARATUS FOR DRAWING WIRE

Filed March 2, 1932

2 Sheets-Sheet 1

Fig. 1.



Fig. 2.



INVENTOR

Paul M. Mueller  
BY  
Emery, Booth, Vane, & Whittlesey  
ATTORNEY

Oct. 29, 1940.

P. M. MUELLER

2,220,048

APPARATUS FOR DRAWING WIRE

Filed March 2, 1932

2 Sheets-Sheet 2

Fig. 3.



Fig. 4.



Fig. 5.



Fig. 6.



INVENTOR

*Paul M. Mueller*

BY

*Emery, Booth, Vaneasy & Whitemore*

ATTORNEY

## UNITED STATES PATENT OFFICE

2,220,048

## APPARATUS FOR DRAWING WIRE

Paul M. Mueller, Rome, N. Y., assignor to General  
Cable Corporation, New York, N. Y., a corpora-  
tion of New Jersey

Application March 2, 1932, Serial No. 596,214

3 Claims. (Cl. 205—14)

This invention relates to apparatus for drawing metal, and pertains particularly to wire drawing.

In the literature of wire drawing, there is occasional reference to a so-called "back pull effect," which is described therein as a phenomenon which increases the drawing tension required if any adverse tension is applied to the wire which is entering the die. Heretofore, such back pull has been considered to be detrimental and therefore to be avoided, because it increased the horse power required for the draft, and in wire drawing in the past it has been the constant effort to minimize or to entirely eliminate back pull.

I have discovered, however, that under certain conditions, instead of being detrimental, back pull can be used to advantage, and that if properly used, instead of increasing the horse power required for the draft, the horse power can be decreased sufficiently to effect substantial savings in the wire drawing operation. In order to take advantage of this effect, however, the back pull must be applied in such manner that its force is applied to some member connected, either mechanically, electrically, or otherwise, with the source of power so that power may be returned to the system without substantial dissipation by frictional or other losses. Preferably the back pull applied should be substantial, and much greater than the ordinary or accidental back pulls which are warned against in the literature because the saving in power increases as the amount of back pull increases. The ideal condition would be that in which the back pull was substantially equal to the tensile strength of the metal, but this is impractical in operation because of lack of any safety factor. In general, therefore, it may be said that best results are obtained when the back pull applied approaches the tensile strength of the metal as nearly as possible, having regard for a proper factor of safety. A back pull of 30,000 pounds per square inch of exit area of the die has been found to give good results in drawing copper, but this figure may vary widely under varying conditions and with different metals. It has been found that if back pull is applied as described herein, the surface friction of the metal as it passes through the die is reduced substantially, and this of course provides a logical explanation of the saving in power, for power is consumed

in overcoming surface friction and internal friction, and even though the internal friction may be unchanged, any saving in surface friction will result in a saving in the power required for the draft.

A preferred embodiment of the invention selected for purposes of illustration is shown in the accompanying drawings, in which:

Figure 1 is a top plan view in semi-diagrammatic form of an apparatus embodying the invention and adapted for a single draft.

Figure 2 is a side elevation of the same.

Figure 3 is a similar top plan view of apparatus adapted for multiple draft work.

Figure 4 is a side elevation also in semi-diagrammatic form. In this figure the numerals and arrows above the figure indicate the tensions and die seat pressures applied at various points in accordance with the illustrative table given hereinafter.

Figure 5 is an enlarged view of one of the capstan shafts, the clutch mechanism being shown in section.

Figure 6 is a section of one of the dies.

Referring to the drawings, the apparatus illustrated in Figures 1 and 2 is a simple form of apparatus embodying the invention in which the wire being drawn is first wound around capstan 1, then passed through die 2, and then wound around capstan 3. The capstans are driven by a motor 4 through capstan shafts 5 and 6 which are connected to the main shaft 7 through properly graduated bevel gears 8 and 9, the capstan 3 being driven at a higher speed than the capstan 2. In the preferred embodiment illustrated capstan 3 is connected to its shaft through a compensating clutch which may take the form illustrated in Figure 5 showing a spring loaded friction clutch in which the sliding sleeve 28 is pressed against the web 29 of the capstan by means of the spring 30. The clutch on shaft 6 is adjusted so as to limit the torque applied to the capstan 3 to a predetermined amount determined as hereinafter set forth. In making this determination the back pull to be applied is first decided. This back pull is multiplied by the exit area of the die in order to obtain the actual value of the back pull in pounds. For example, if it is decided to apply a back pull of 30,000 pounds per square inch, and the exit area of the die is .00647 square

inch, the back pull or tension on the wire between the capstan 1 and die 2 would be 194 pounds. The amount of resistance to passage of the wire through the die or "die seat pressure" is determined next by actual test, and by adding this amount to the back pull, a value is obtained which represents the amount of forward pull which is required. Thus in the above example, the die seat pressure is found to be 92 pounds, which, added to the back pull gives the sum of 286 pounds which is the required forward pull. The torque applied to the capstan is therefore limited to this amount, and the clutch is adjusted accordingly.

Following through the above example and calculating the horsepower required if the capstans 1 and 3 are geared to run at 1390 feet per minute and 1750 feet per minute respectively, we find:

Ft. lbs.  
per minute

20 Work applied at capstan 3  $286 \times 1750 = 500,000$   
Work applied at capstan 1  $194 \times 1390 = 269,000$

Differential work supplied by motor  $231,000$

25 As compared with this, it is found experimentally that in the absence of back pull, the forward pull required to draw the same wire through the same die is 191 pounds. Again calculating the horsepower required, we find:

30  $191 \times 1750 = 334,000$  ft. lbs. per minute

Thus the horsepower required in the second case is more than 40% greater than that required in the first case where back pull is applied.

35 The same principles may be applied with com-

must be applied by the capstan 13. The back pull from the next succeeding die 13 is applying a forward pull of 194 pounds to the capstan. Therefore, it is only necessary to apply a torque through the capstan shaft equivalent to a pull of 144 pounds, and the clutch is adjusted in such manner that this amount shall not be exceeded. Thus, the torque applied to each capstan shaft except the last is less than sufficient to pull the wire through the preceding die, and the back pull of the next succeeding die is relied upon to make up the deficiency. If for any reason the torque applied tends to increase above the predetermined amount, the clutch will slip, of course. It will be understood, of course, that in place of a common drive from a single source of power, each capstan shaft might be driven by a separate constant torque motor.

It will also be understood that in practice, one of the capstans in the series, as for example capstan 17, may be locked to its shaft by setting up on the clutch or in any other convenient manner. This is advisable in order to provide proper wire speed control.

As an example of the saving which may be made in multiple draft work by utilizing back pull in the manner described, an actual comparison between the practice described herein and old wire drawing practice will be given.

The example used is a reduction of annealed wire from size .128 to size .064 in one continuous draft in six dies. The following table illustrates the determination of power required in a case where back pull is used in accordance with the present method:

| Size | Exit area of die | Back pull in pounds | Die seat pressure | Forward pull in pounds | Resultant forward pull in pounds | Velocity in feet per minute | Power in foot pounds per minute |
|------|------------------|---------------------|-------------------|------------------------|----------------------------------|-----------------------------|---------------------------------|
| .128 | .01297           |                     |                   |                        |                                  |                             |                                 |
| .114 | .01028           | 0                   | 216               | 216                    | -29                              | 1,100                       | -32,800                         |
| .102 | .00815           | 245                 | 93                | 338                    | 144                              | 1,390                       | 200,000                         |
| .091 | .00647           | 194                 | 92                | 286                    | 132                              | 1,750                       | 231,000                         |
| .081 | .00513           | 154                 | 82                | 236                    | 114                              | 2,200                       | 251,000                         |
| .072 | .00407           | 122                 | 70                | 197                    | 100                              | 2,780                       | 278,000                         |
| .064 | .00322           | 97                  | 60                | 157                    | 157                              | 3,500                       | 555,000                         |
|      |                  |                     |                   |                        |                                  |                             | 1,483,000                       |

parable results in the case of the multiple draft apparatus illustrated in Figures 3 and 4. In this case, the apparatus comprises a plurality of dies 10, 12, 13, 14, 15 and 16 and a plurality of capstans 17, 18, 19, 20, 21 and 22. The wire to be drawn is first passed through die 10, then several turns are taken around capstans 17, then the wire is passed through a die 12 and around capstan 18 and so on through the entire series of dies. As illustrated, the capstans are all driven by a motor 23 which is connected to a main shaft 24 having mounted thereon bevel gears 25 of properly graduated sizes which mesh with bevel gears 26 on the capstan shafts 27. Each of the capstans is connected to its drive shaft 27 through a compensating clutch such as that illustrated in Figure 5 and in each case, the clutch is adjusted in such manner that the torque applied to the capstan by its shaft is equal to the required forward pull, less the back pull for the next succeeding die. The reason for this deduction will be clear when it is realized that the back pull for the next succeeding die is applied as a forward pull on the preceding capstan. Thus, referring, for example, to Figures 3 and 4, the forward pull required to pull the wire through die 12 is 338 pounds. This pull

In the above table, as in the single draft example, the back pull applied is 30,000 pounds per square inch of exit area of each die. Thus the "Back pull in pounds" is obtained by multiplying 30,000 pounds by the exit area of each die. The values for "Die seat pressure" are determined experimentally, and the values for "Forward pull in pounds" are obtained by adding the back pull to the die seat pressure. The "Resultant forward pull in pounds" is the difference between the forward pull and the back pull for the next succeeding die. This value, as previously explained, determines the torque which must be applied to each capstan shaft. The power is obtained by multiplying the resultant forward pull by the velocity.

In the above table, and in the machine illustrated in Figures 3 and 4 it will be noted that no back pull is applied at die 10. It will be understood, of course, that if desired, an additional capstan could be placed ahead of the die 10 in the same manner that the capstan 1 is placed ahead of the die 2 in Figures 1 and 2, with a further saving in power. But whereas in the single draft machine this capstan is essential, in the multiple draft machine its use is optional, and in many installations the saving from its use

in proportion to the total saving may not be sufficient to warrant the extra complication. The above table, however, in comparison with the table about to be given, shows the large saving to be had even without the use of the extra capstan.

For purposes of comparison, the next table gives the comparable figures for the same reduction, but without utilizing the back pull effect.

| 10 | Size | Exit area of die | Die seat pressure | Forward pull in pounds | Velocity in feet per minute | Power in foot pounds per minute |
|----|------|------------------|-------------------|------------------------|-----------------------------|---------------------------------|
| 16 | .128 | .01297           | 0                 | 0                      | 875                         | 0                               |
|    | .114 | .01028           | 216#              | 216#                   | 1,100                       | 237,000                         |
|    | .102 | .00815           | 212               | 212                    | 1,390                       | 295,000                         |
|    | .091 | .00647           | 191               | 191                    | 1,750                       | 334,000                         |
|    | .081 | .00513           | 164               | 164                    | 2,200                       | 361,000                         |
|    | .072 | .00407           | 134               | 134                    | 2,780                       | 373,000                         |
| 20 | .064 | .00322           | 110               | 110                    | 3,500                       | 385,000                         |
|    |      |                  |                   |                        |                             | 1,985,000                       |

In the above table the die seat pressures are also determined experimentally, but since back pull is eliminated, the forward pull is equal to the die seat pressure in each case. The power required is again calculated by multiplying forward pull by the velocity. As will be observed, the total power required in the second table is 33 1/3% greater than the power required in the first table where back pull is used in accordance with the principles of the invention.

It will be understood, of course, that the above tables are merely illustrative of the results obtainable under the conditions assumed. With other conditions the results will vary, but a saving in power will result uniformly if the back

pull applied is utilized in accordance with the principles described herein. Wear on the dies is also materially reduced by this method.

It has been observed that wire drawn in accordance with the above described invention 5 possesses a somewhat greater tensile strength than wire drawn by ordinary methods.

It will be understood that the invention may be variously modified and embodied within the scope of the subjoined claims.

I claim as my invention:

1. A wire drawing machine comprising a plurality of dies, a plurality of capstans, common means for driving said capstans, the connections between said capstans and said common driving means including means for limiting the torque applied to each capstan by the common driving means to an amount less than sufficient to pull the wire through the preceding die.

2. A wire drawing machine comprising, in combination, a plurality of dies, a plurality of capstans located between said dies, a common shaft for driving said capstans, and means for limiting the torque applied by said drive shaft to each capstan to an amount less than sufficient to draw 25 the wire through the die immediately preceding the capstan.

3. A wire drawing machine comprising a die, a capstan for pulling wire through the die, a second capstan for exerting a back pull on the wire as 30 it is drawn through the die, common means for driving said capstans, and means for limiting the torque applied to the first mentioned capstan to an amount less than sufficient to draw the wire through the die in the absence of back 35 pull on the wire.

PAUL M. MUELLER.